

## UNITED STATES PATENT OFFICE

2,378,437

## ALLOY STEEL

Byramji D. Saklatwalla, Pittsburgh, Pa.

No Drawing. Application January 19, 1943,  
Serial No. 472,855

5 Claims. (Cl. 75—125)

This invention relates to an alloy steel intended for structural purposes and possessing in the as-rolled state high strength and corrosion resistance. My steel is low in carbon and silicon contents, with a comparatively low manganese content, and containing chromium, nickel, copper, molybdenum and phosphorus as the effective alloying constituents. The chromium, nickel, and molybdenum are employed as strength-imparting agents in the steel and when employed in properly balanced proportions to each other and to the other strength-imparting elements, phosphorus and copper, are found to impart strength without impairing the ductility of the steel, as would be the case were the strength obtained from appreciable contents of carbon, silicon and/or manganese, which are the usual strength-imparting elements in carbon or alloy steels. Contents of chromium, copper, phosphorus, nickel, and molybdenum are incorporated in the steel, in certain selected ranges, such as to impart to the steel a high degree of corrosion resistance. All the elements are used in such balanced proportions that simultaneously strength and corrosion resistance of a high degree are obtained in the steel, permitting reduction of sections and total weight, without sacrifice of life of structures constructed of the steel.

In the older high-strength corrosion-resistant copper-phosphorus steels containing chromium or those containing chromium and molybdenum or nickel and molybdenum, their high strength properties are obtained essentially by the presence of an appreciable silicon content, specified to be from .25 or .35% up to 2 and even up to 3%. Such high silicon steels require particular care during their melting and refining in the open-hearth furnace, and in the process of casting soaking and heating of their ingots prior to the rolling operation. Such extra care is essential in order to obtain the finished rolled steel with a clean structure and in a seam-free and good surface condition. Moreover, high silicon steels are usually produced by casting the ingots with hot-tops entailing extra time and cost in their production. If, to obviate these deficiencies, the silicon content of the steel is lowered, the required strength properties are not obtained, the silicon being the essential strength-imparting element in such steels.

I obviate the above deficiencies and produce by my invention a corrosion-resistant copper-phosphorus steel, although low in silicon, manganese, and carbon, yet with high tensile strength and yield point and capable of being produced by the

open-hearth process practically with equal facility as ordinary low-carbon steel. I accomplish this by incorporating in the copper-phosphorus steel a combination of chromium, nickel, and molybdenum within certain definite ranges. When chromium alone with copper and phosphorus is used, as in the older steels, the requisite tensile strength and yield point are not obtained unless the high percentage of silicon (.25 to 3.0%) is present. Similarly, when chromium and molybdenum alone, or nickel and molybdenum alone, are used with copper and phosphorus, the high percentage of silicon (.35 to 2.0%) has to be present in the steel to obtain the specified strength properties. If nickel alone is used with copper and phosphorus, the amount of nickel necessary to obtain the strength is so high as to make the steel unduly expensive. If with a smaller amount of nickel, a large percentage of copper, such as would be necessary to obtain the strength, is used, the steel becomes subject to precipitation hardening when cooled from a high temperature and possesses a low degree of formability and workability. If a high manganese content, over .5 and up to 1.25% manganese, is used to impart strength to copper-phosphorus steels, such manganese content curtails ductility and especially the impact resistance of the steel, at the same time making it difficultly weldable, owing to the hardening action of the manganese when cooling from welding temperature.

By my composition, in which the percentages of the various alloying elements are used in balanced proportions against one another, I obtain a corrosion-resistant steel which has all the well-known manufacturing advantages of a low-silicon open-hearth steel, such as easy melting and refining and ingot-casting practice. Moreover, with this ease in manufacturing, the steel possesses a higher degree of ductility, impact resistance, and weldability than the high silicon and/or high manganese steels, at the same time displaying strength properties equal to those of such steels. Furthermore, the elements chromium, nickel, copper, molybdenum and phosphorus are used in my steel in such combinations and proportions as to impart to the steel a corrosion resistance several times greater than that of ordinary carbon or copper-bearing steel, enabling it to withstand corrosive conditions to which structural steels are ordinarily subjected in use. I have found that when the elements are used in the specified ranges, the best balance of strength,

ductility, good impact and corrosion resistance are obtained in the finished steel.

For the production of steel of my invention, I use the elements carbon, silicon, manganese, phosphorus, chromium, nickel, molybdenum, and copper within the following general ranges.

|            | Per cent             |
|------------|----------------------|
| Carbon     | .01 to less than .14 |
| Silicon    | .01 to less than .18 |
| Manganese  | .05 to less than .50 |
| Phosphorus | .07 to .18           |
| Chromium   | .25 to 1.5           |
| Nickel     | .25 to 1.25          |
| Molybdenum | .07 to .60           |
| Copper     | .18 to .75           |

The following is a more restricted range of elements for the production of the steel:

|            | Per cent   |
|------------|------------|
| Carbon     | .05 to .13 |
| Silicon    | .01 to .12 |
| Manganese  | .15 to .45 |
| Phosphorus | .08 to .15 |
| Chromium   | .35 to 1.0 |
| Nickel     | .30 to .90 |
| Molybdenum | .08 to .35 |
| Copper     | .25 to .65 |

A still more restricted range within which steels of well balanced properties can be produced is as follows:

|            | Per cent   |
|------------|------------|
| Carbon     | .06 to .12 |
| Silicon    | .03 to .10 |
| Manganese  | .20 to .40 |
| Phosphorus | .08 to .13 |
| Chromium   | .40 to .85 |
| Nickel     | .40 to .75 |
| Molybdenum | .10 to .30 |
| Copper     | .30 to .60 |

I prefer to keep the manganese content low, as I have found that any substantially high manganese content of the steel is deleterious, inasmuch as it lowers the impact resistance and weldability of the steel. The manganese content of the steel must be maintained below a maximum of .5%.

The sulphur content should be low, as in good steel-making practice, in which it is under .05%. I prefer that the sulphur content be as low as possible, preferably under .03%.

The balance of my composition is made up of commercial steel with the usual impurities derived from the raw materials used in the making of the steel, such as ore, fuel, fluxes, scrap, etc. If desired, the steel can be treated with the usual deoxidizing and refining agents, such as aluminum, ferro-titanium, ferro-zirconium, ferro-vanadium, ferro-boron, etc., or with the complex deoxidizers, such as silicon-calcium, silicon-aluminum-calcium, silicon-zirconium-calcium, or with the so-called "intensifier" agents containing a plurality of refining elements.

The steel of my composition, owing to its low carbon and silicon contents, possesses a high degree of ductility relative to its strength, together with the high impact resistance, due to its strength being derived from the chromium, nickel, and molybdenum in combination with the phosphorus and copper. The steel possesses an average tensile strength of between 60,000 and 75,000 lbs. per square inch, with an average yield point of between 45,000 and 60,000 lbs. per square inch, together with a minimum elongation of 22%

in two inches based on a 2-inch gage length specimen. Practically all the steels falling within the above ranges of composition are capable of meeting the usual commercial specifications for high tensile steels; namely, over 70,000 lbs. per square inch tensile strength and over 50,000 lbs. per square inch yield point. The steels possess an Izod value generally of about 40 foot-pounds or over. They possess good welding, bending and forming properties. It is an essential characteristic of the steel that it possess low hardenability, so that in the process of welding, hardening adjacent to the weld does not take place. These properties are obtained in the steel in the as-rolled condition without any expenditure for heat treatment which is an important economic advantage.

The elements nickel, molybdenum, and copper used in my steel being not oxidizable are fully recovered from the scrap. Owing to the recovery of these expensive elements from the scrap, and as no heat treatment is required to obtain the desirable balanced properties of the steel, it being used in the as-rolled condition, the fabrication of welded structures such as railroad cars, ships and other transportation units can be accomplished with this steel at a relatively cheap cost.

The steel of my invention can be produced by the ordinary steel-making processes, such as the open-hearth, electric furnace, or converter process. The nickel, copper, and molybdenum can be added in the furnace, during the melting and refining of the steel, according to the usual practice. The chromium, as ferro-chrome, and the phosphorus, as ferro-phosphorus, can be added in the furnace, but it is preferable to add them in the ladle after tapping the steel to avoid unnecessary loss of these elements through oxidation and to more easily control their content in the finished steel.

I claim:

1. A corrosion resistant, low-carbon, low-alloy high strength steel with silicon and manganese contents not in excess of those found in mild carbon steel, and being under the contents required for imparting added strength to carbon steels, the silicon being less than about .18% and the manganese less than about .50%, together with a carbon content of from .01% to less than .14%, containing as essential alloying constituents chromium from .25% to 1.5%, nickel from .25% to 1.25%, molybdenum from .07% to .60%, copper from .18% to .75%, and phosphorus from .07% to .18%, the balance being commercial steel, and characterized in the as-rolled condition by both high tensile and high yield strengths, together with a greater degree of ductility and impact resistance than is found in copper-phosphorus steel of equivalent tensile strength and containing silicon in excess of .18% or manganese in excess of .50%.

2. A corrosion resistant, low-carbon, low-alloy high strength steel with silicon and manganese contents not in excess of those found in mild carbon steels, and being under the contents required for imparting added strength to carbon steels, the silicon being less than about .12% and the manganese less than about .45%, together with a carbon content of from .05% to less than .13%, and containing as essential alloying constituents chromium from .35% to 1.0%, nickel from .30% to .90%, molybdenum from .08% to .35%, copper from .25% to .65%, and phosphorus from .08% to .15%, the balance being commercial steel, and characterized in the as-

rolled condition by both high tensile and high yield strengths, together with a greater degree of ductility and impact resistance than is found in copper-phosphorus steel of equivalent tensile strength and containing silicon in excess of .18% or manganese in excess of .50%.

3. A corrosion resistant, low-carbon, low alloy high strength steel with silicon and manganese contents not in excess of those found in mild carbon steels, and being under the contents required for imparting added strength to carbon steels, the silicon being less than about .10% and the manganese less than about .40%, together with a carbon content of from .06% to .12%, and containing as essential alloying constituents 15 chromium from .40% to .85%, nickel from .40% to .75%, molybdenum from .10% to .30%, copper from .30% to .60%, and phosphorus from .08% to .13%, the balance being commercial steel, and characterized in the as-rolled condition by both 20 high tensile and high yield strengths, together with a greater degree of ductility and impact resistance than is found in copper-phosphorus steel of equivalent tensile strength and containing silicon in excess of .18% or manganese in 25 excess of .50%.

4. A corrosion resistant, low-carbon, low-alloy high strength steel with silicon and manganese contents not in excess found in mild carbon steels, the silicon being less than about .18% and the manganese less than about .50%, together with a carbon content of less than about .14%, and containing as essential alloying constituents 10 chromium from .25% to 1.5%, nickel from .25% to 1.25%, molybdenum from .07% to .60%, copper from .18% to .75%, and phosphorus from .07% to .18%, the balance being commercial steel, and characterized in the as-rolled condition by a relatively high ratio of ductility to tensile strength.

5. A corrosion resistant, low-carbon, low-alloy high strength steel containing as essential alloying constituents chromium from .25% to 1.5%, nickel from .25% to 1.25%, molybdenum from .07% to .60%, copper from .18% to .75%, and phosphorus from .07% to .18%, together with 15 carbon from .01 to less than .14%, silicon from .01 to less than .18%, and manganese from .05 to less than .50%, the balance being commercial steel.

BYRAMJI D. SAKLATWALLA.